

Sept. 26, 1972

W. R. MOHONDRO ET AL

3,694,272

METHOD FOR FORMING ALUMINUM SHEET

Filed Dec. 24, 1970



WILLIAM R. MOHONDRO *sgd*  
MAURICE C. FETZER  
INVENTORS

BY *Edward J. Lynch*  
ATTORNEY

## 1

3,694,272

**METHOD FOR FORMING ALUMINUM SHEET**  
William R. Mohondro, Dublin, and Maurice C. Fetzer,  
Walnut Creek, Calif., assignors to Kaiser Aluminum &  
Chemical Corporation, Oakland, Calif.  
Filed Dec. 24, 1970, Ser. No. 101,239  
Int. Cl. C21d 7/14, 9/00

U.S. Cl. 148—12.7

13 Claims

**ABSTRACT OF THE DISCLOSURE**

A process for the production of thin Al-Zn-Mg sheet material from relatively thick stock, wherein the sheet material undergoes a substantial reduction in thickness with no tendency for edge cracking or tearing, comprising solution heat treating the relatively thick sheet, cold rolling the sheet so as to produce a reduction in thickness between 40% and 75%, preferably between 50% and 70%, artificially aging the sheet, and cold rolling the sheet to the final desired gauge thickness. According to one embodiment of the invention, the solution heat treatment step comprises controlling the temperatures during hot rolling to effect a dissolution of substantially all of the alloying constituents and then quenching the sheet before it is coiled.

**BACKGROUND**

The present invention relates to a process for making Al-Zn-Mg sheet from relatively thick stock without cracking or tearing during subsequent cold rolling operations.

Prior methods for forming thin Al-Zn-Mg alloy sheet include cold rolling the hot rolled intermediate product to final gauge, solution heat treating and subsequently aging the sheet. Due to the high work hardening rates of these alloys, it was frequently necessary to provide one or more anneals for stress relief during the cold rolling operations. Moreover, due to the high temperatures of the solution heat treatment step, the sheet material in the final gauge thickness becomes distorted and the surface finish is impaired which requires corrective procedures known to the art. The hot rolling operations usually reduce the sheet thickness to between about 0.08 and 0.20 inch. Sheet material having a thickness greater than 0.20 inch is difficult to coil and sheet material thinner than 0.08 inch is usually not strong enough to be hot rolled without tearing. The final cold-rolled sheet thickness depends upon product use but usually ranges from 0.005 to 0.06 inch.

The solution heat treating process is herein defined as heating above a temperature at which substantially all of the age hardening alloy elements are in solid solution in the aluminum matrix, i.e., above the solvus temperature and then quenching to freeze the alloying constituents in solid solution. When the solution heat-treated alloy is heated to an elevated temperature, the alloying constituents precipitate from solid solution, thus increasing the strength and hardness of the material. The technique of artificial aging of heat-treatable aluminum alloys to which the present invention pertains is well known to those skilled in the art.

**SUMMARY OF INVENTION**

The present invention relates to a method by which thin sheet of an aluminum alloy containing zinc and magnesium as the principle alloying additives can be made without the tearing or cracking of the sheet during the cold rolling operation, and, moreover, which will possess sufficient ductility in the final product to be further fabricated into such items as embossed roofing sheet, siding, can bodies, can ends, and the like.

## 2

The method of the present invention comprises solution heat treating a relatively thick aluminum-zinc-magnesium sheet material, usually between 0.08-0.20 inch thick, cold rolling the sheet so as to produce a reduction in thickness of between 40% and 75%, preferably between 50% and 70%, artificially aging the sheet and cold rolling the sheet to the desired gauge. By controlling the degree of deformation during initial cold rolling and by artificially aging the sheet thereafter, the metal exhibits little or no tendency to work harden during the final cold rolling operation. The process of the present invention is directed toward an aluminum alloy consisting essentially of 4.0-6.0% zinc, 0.7-3.0% magnesium, up to 2.5% copper, up to 0.6% manganese and balance aluminum, incidental elements and normal impurities.

**DESCRIPTION OF THE DRAWINGS**

FIGS. 1A and 1B are graphical representations which show the effect of the percent cold rolling after aging on the tensile properties of the sheet at various levels of reduction in cold rolling prior to aging.

**DETAILED DESCRIPTION OF THE INVENTION**

The present invention is directed toward the process of treating an aluminum base alloy consisting essentially of 4.0-6.0% zinc, 0.7-3.0% magnesium, up to 2.5% copper, up to 0.6% manganese, and the balance aluminum, incidental elements and normal impurities. The expression "incidental elements and normal impurities," as used herein, includes iron, 0.35% maximum; silicon, 0.30% maximum; titanium, 0.10% maximum; chromium, 0.25% maximum; zirconium, 0.25% maximum; other elements 0.05% each maximum, 0.15% total maximum. More specifically, the present invention is directed to the production of sheet material having a composition consisting essentially of 4.8-5.4% zinc, 0.95-1.3% magnesium, 0.15-0.40% manganese, less than 0.10% copper, less than 0.08% chromium, less than 0.08% zirconium, the sum of the chromium and zirconium not exceeding 0.10%, and the balance aluminum, incidental elements and normal impurities.

According to the present invention, after the normal pretreatments such as homogenizing, scalping, initial breakdown and the like, the alloys of the present invention are hot rolled to a desired intermediate gauge, normally between about 0.08 and 0.15 inch, solution heat-treated, cold rolled so as to produce a reduction thickness between about 40-75%, artificially aged and then cold rolled to the thickness desired. The solvus temperature for the alloys of this invention is from about 610° F. to 734° F., and thus the solution temperature must exceed 610° F. However, the temperature of the solution heat treatment should be below the temperature at which any of the alloying phases becomes molten. For the chromium- and zirconium-free alloys, i.e., containing less than 0.10% chromium and/or zirconium, the quench rate during the solution heat treatment is not particularly critical. For example, the chromium- and zirconium-free material can be quenched using a cold or water spray, forced air and the like. Generally, however, for all the alloys of this invention cooling rates should be greater than 5° F. per second, at least between the solvus temperature and 450° F. The artificial aging is conducted at a temperature between about 150° F. and 350° F. for a period from about 6 to 72 hours. Single or multiple temperature aging practices can be employed.

According to one particularly advantageous embodiment of the present invention, the temperatures in the hot rolling step are controlled so as to put into or maintain in solution the alloying constituents during hot rolling and quenching the sheet material to freeze the alloying constituents in solution prior to coiling of the hot-rolled sheet. This em-

bodiments is particularly directed to the chromium- and zirconium-free alloy composition because these alloys are particularly insensitive to quench rate. For a successful solution heat treatment using this approach, it is necessary for the metal entering the hot rolling mill to be at a temperature above the solvus temperature for the alloy, i.e., greater than 610° F. The hot-rolled sheet generally is quenched coming off a hot rolling mill although the quenching can occur during the hot rolling operation itself. Because this alloy is not quench sensitive, a wide variety of quenching mediums can be used. For example, water sprays, soluble oil sprays, air blasts and the like. This approach is particularly advantageous from an economic standpoint in that an additional solution heat treat step is eliminated. However, all of the hot-rolled sheet material of this invention should be cooled below 300° F., preferably below 275° F., before coiling. The material has a tendency to age soften during storage if coiled at high temperatures. The quench sensitive alloys can be utilized in this procedure but the quenching rate must be quite high, i.e., greater than 275° F. per second at least in the range between the solvus temperature and 550° F., and the sheet must be maintained at a temperature above the solvus temperature until the sheet is quenched.

The present invention uniquely provides for an economical and easily controlled method for producing thin sheet material which does not crack or tear with substantial reductions in thickness during cold rolling. In accordance with this invention it has been found that by controlling the amount of cold rolling before aging, the sheet material has substantially no tendency to work harden upon subsequent cold rolling. The cold rolling after solution heat treatment but before aging is controlled to effect a thickness reduction from about 40 to 75%. By so doing, the sheet material exhibits no substantial increase in tensile or yield strength even though the material is subjected to large additional amounts of cold rolling, e.g., up to 70% or more.

If the alloys of the present invention are cold rolled before aging, herein termed preworked, substantially less than 40%, the sheet material will work harden to considerable extents during subsequent cold rolling. In addition, if the alloys are preworked more than about 75%, the sheet material has a tendency to crack and tear during pre-work. After a controlled amount of prework and aging the sheet material of the present invention can be subjected to extremely large amounts of cold rolling, herein termed postworked, with no tendency to work harden. Moreover, the postworked sheet material can easily be fabricated into other forms without the expensive corrective treatments required by the prior art processes such as straightening, surface finishing, and the like.

It has been found that a microstructure is developed during the initial cold rolling of the present invention which is characterized by intragranular deformation banding patterns. The deformation bands serve as precipitation sites during the subsequent aging treatment. The volume fraction, interparticle spacing and size of the precipitated age hardening phases of the present invention are substantially larger than those found when the alloy is aged with no substantial prework. Moreover, the precipitated phases are substantially noncoherent, which are to be distinguished from the highly coherent phases which are precipitated when the alloy is not preworked by substantial amounts. It is believed that due to the above factors the degree of cross-slip, the material of the present invention can accommodate remains substantially constant and therefore the work hardening rate is negligible.

The increases in tensile strength and yield strength normally experienced with the present invention are less than 15%. Increased amounts of prework and smaller amounts of copper, preferably less than 0.10%, provide for smaller increases in work hardening rates.

The following is an example of an embodiment of the present invention, which is intended to be illustrative and to demonstrate the invention rather than to limit it.

The process of the present invention was applied to an aluminum alloy sheet material which had been hot rolled to the intermediate gauge of 0.114 inch. The sheet had the following composition:

|    | Percent |
|----|---------|
| Zn | 5.20    |
| Mg | 1.23    |
| Mn | 0.26    |
| Si | 0.10    |
| Fe | 0.25    |
| Cr | 0.02    |
| Cu | 0.05    |
| Ti | 0.02    |
| Al | Balance |

The sheet material was solution heated to 750° F. and maintained at that temperature for 30 minutes followed by quenching. After two days at room temperature, separate samples of the sheet material were cold rolled, or preworked, 0%, 50% and 70%. After initial cold rolling, the sheet was artificially aged using an aging practice of 195° F. for 8 hours followed by 300° F. for 8 hours. Following the aging treatment, separate samples of the preworked sheet material which had been cold rolled 0%, 50% and 70% were postworked by cold rolling 40%, 60% and 70% of the preworked thickness. The various samples were tested for both tensile and yield strengths as well as for bendability. The results are given in Table I. The tensile tests vs. percent of postwork is also shown in FIGS. 1A and 1B. The bend test involves bending a specimen 180° over progressively smaller mandrels until the specimen breaks. The results are given in the diameter of the bend in terms of the thickness of the sheet.

|    | Pre-work, percent | Post-work, percent | Before aging        |                   | After aging         |                   | Sheet thickness, in. |
|----|-------------------|--------------------|---------------------|-------------------|---------------------|-------------------|----------------------|
|    |                   |                    | Tensile str. K.s.i. | Yield str. K.s.i. | Tensile str. K.s.i. | Yield str. K.s.i. |                      |
| 40 | 0                 | 0                  | 51.2                | 28.7              | 56.7                | 50.4              | .114                 |
|    | 40                | 40                 |                     |                   | 68.3                | 63.8              | .073                 |
|    | 70                | 70                 |                     |                   | 71.5                | 67.6              | .058                 |
|    | 0                 | 0                  |                     |                   | 72.4                | 68.9              | .0348                |
|    | 40                | 40                 |                     |                   | 55.5                | 51.9              | .058                 |
|    | 60                | 60                 | 65.1                | 56.0              | 56.5                | 54.4              | .0351                |
| 50 | 70                | 70                 |                     |                   | 58.0                | 56.1              | .0228                |
|    | 0                 | 0                  |                     |                   | 59.1                | 57.2              | .0177                |
|    | 40                | 40                 |                     |                   | 56.8                | 53.7              | .0348                |
|    | 60                | 60                 | 68.9                | 61.3              | 56.7                | 54.7              | .0211                |
| 45 | 70                | 70                 |                     |                   | 57.1                | 54.9              | .0148                |
|    | 0                 | 0                  |                     |                   | 58.0                | 55.9              | .0109                |

From the test data it is evident that when the sheet material is subjected to the process of the present invention, the sheet material does not substantially work harden upon subsequent cold rolling even when substantial reductions in thickness occur and, furthermore, the resultant product is easily fabricated into other shapes.

What is claimed is:

1. The process of making thin Al-Zn-Mg alloy sheet from relatively thick stock comprising
  - (a) solution heat treating relatively thick aluminum alloy sheet having a composition consisting essentially of about 4.0 to 6.0% zinc, about 0.7 to 3.0% magnesium, up to 2.5% copper, up to 0.6% manganese and the balance aluminum, incidental elements and normal impurities;
  - (b) cold rolling said sheet so as to produce a reduction in thickness thereof between about 40 and 75%;
  - (c) artificially aging said cold-rolled sheet at a temperature between about 150° F. and 350° F. for a period between about 6 to 72 hours; and
  - (d) cold rolling said artificially aged sheet to the final gauge.
2. The process of claim 1 wherein the sheet has a composition consisting essentially of 4.8 to 5.4% zinc, 0.95 to 1.3% magnesium, 0.2 to 0.45% manganese, less than 0.10% copper and the balance aluminum, incidental elements and normal impurities.

3. The process of claim 1 wherein said sheet contains less than 0.08% chromium and less than 0.08% zirconium.

4. The process of claim 1 wherein said sheet contains less than 0.10 copper.

5. The process of claim 1 wherein said relatively thick sheet is solution heated at a temperature above about 610° F.

6. The process of claim 4 wherein said relatively thick sheet is quenched at a rate greater than 5° F. per second from the solvus temperature to below about 450° F.

7. The process of claim 1 wherein said cold rolling before aging produces a reduction in thickness between about 50% and 70%.

8. The process of making thin Al-Zn-Mg alloy sheet 15 from relatively thick stock comprising

(a) preheating said aluminum alloy stock, having a composition consisting essentially of about 4.0 to 6.0% zinc, about 0.7 to 2.0% magnesium, less than 0.10% copper, up to 0.6% manganese and the balance aluminum, incidental elements and normal impurities, to above the solvus temperature thereof;

(b) hot rolling said thick stock with the mill entry temperature of said stock being above the solvus temperature for said composition;

(c) quenching said hot-rolled sheet to maintain substantially all of the alloying constituents in solid solution;

(d) cold rolling said hot-rolled sheet so as to produce a reduction in thickness thereof between about 40% and 75%;

(e) artificially aging said cold-rolled sheet at a tem-

perature between about 150° F. and 350° F. for a period between about 6 to 72 hours; and

(f) cold rolling said artificially aged sheet to the final gauge.

5. 9. The process of claim 8 wherein the hot-rolled sheet is coiled at a temperature below 300° F.

10. 10. The process of claim 8 wherein the cooling rate during quenching as at least 5° F. per second from the solvus temperature to below about 450° F.

10. 11. The process of claim 8 wherein the sheet has a composition consisting essentially of 4.8 to 5.4% zinc, 0.95 to 1.3% magnesium, 0.2 to 0.45% manganese, less than 0.10% copper and the balance aluminum, incidental elements and normal impurities.

10. 12. The process of claim 6 wherein said sheet contains less than 0.08% chromium and less than 0.08% zirconium.

10. 13. The process of claim 8 wherein the mill entry temperature is between about 610° F. and 740° F.

#### References Cited

#### UNITED STATES PATENTS

|           |         |                        |            |
|-----------|---------|------------------------|------------|
| 3,580,747 | 5/1971  | Howitt et al. -----    | 148—12.7   |
| 3,542,606 | 11/1970 | Westerman et al. ----- | 148—12.7   |
| 3,329,537 | 7/1967  | Loach -----            | 148—11.5 X |
| 3,346,372 | 10/1967 | Jagaciak -----         | 148—11.5 X |
| 2,506,788 | 5/1950  | Hobbs -----            | 148—12.7   |

L. DEWAYNE RUTLEDGE, Primary Examiner

G. K. WHITE, Assistant Examiner